

May 29, 1928.

1,671,413

D. C. DICKSON

METHOD OF PREVENTING SLAG SURGE IN THERMITE WELDING PRACTICE

Filed Sept. 1, 1925



Fig. 2.



Fig. 2.

Inventor

D. C. Dickson

By Chas. J. Wayne

Attorney

Patented May 29, 1928.

1,671,413

## UNITED STATES PATENT OFFICE.

DONALD CAMERON DICKSON, OF JERSEY CITY, NEW JERSEY, ASSIGNOR TO METAL & THERMIT CORPORATION, OF CARTERET, NEW JERSEY, A CORPORATION OF NEW JERSEY.

### METHOD OF PREVENTING SLAG SURGE IN THERMITE WELDING PRACTICE.

Application filed September 1, 1925. Serial No. 53,948.

The invention relates to a novel method of preventing the surging of the slag within the mold in thermite welding practice, in which the elements to be welded by the 5 molten thermite metal are enclosed in a mold and the superheated molten thermite metal is teemed into the mold from a crucible located above the same, the method comprising the teeming of substantially all of the 10 molten metal directly into the pouring gate of the mold and then diverting the portion of the molten stream containing the slag from the gate entrance by relative lateral movement of the crucible and mold, so that 15 the falling slag stream will not impact the molten metal within the mold.

The operation of the invention is illustrated in the accompanying drawings, in which:

20 Fig. 1 is a sectional elevation of a mold with the crucible in its initial pouring position relative to the pouring gate.

Fig. 2 is a similar view showing the final position of the crucible.

25 Referring to the drawings, 1 indicates a typical mold, having a preformed cavity 2 into which the ends of the rails to be welded extend, the cavity receiving the superheated molten metal discharged from the bottom 30 of crucible 4, which is directed into said cavity by a pouring gate 3.

In alumino-thermic welding, more particularly in welding the ends of rails, effected by tapping highly heated thermite metal, such 35 as steel, from a crucible, into a mold containing the parts to be welded, it has been found that the highly molten slag, which floats on the molten steel in the crucible, frequently gains access to the interior of the mold and 40 comes in contact with the surfaces to be welded, resulting in weakened and imperfect welds due to the adhesion of the slag to the metal. It has been found that the entrance of the slag into the mold cavity is 45 due to the surge set up by the falling stream of molten slag into the mold cavity, after the thermite steel has entered and substantially filled the mold. It has been proposed heretofore to prevent this surging of the 50 slag by pouring the molten stream containing the slag upon an angularly disposed wall of the pouring gate to dissipate the force

of falling slag impacting the same. In rail welding practice, however, the dimensions of the mold are reduced to the minimum and 55 the small top surface of the mold contains numerous gates, risers and vent holes, leaving little or no room for the provision of an inclined pouring surface adjacent the upper portion of the pouring gate. Furthermore, 60 in the use of such small quantities of thermite as is employed in rail welding, it frequently happens that the molten stream does not fall exactly vertically downward and it is more or less difficult to direct the stream onto any 65 particular part of the mold, with any great accuracy. In order to avoid these difficulties, and nevertheless to overcome the very objectionable slag surge and trapping within the mold, I have found it sufficient to deflect 70 the falling stream of molten material from direct entrance into the pouring gate by moving the mold and crucible relatively, in a lateral direction, as soon as the mold has been substantially filled with steel and before 75 the slag containing portion of the charge has had an opportunity to enter the pouring gate. This relative lateral movement of the crucible and mold need not be extensive, but should be sufficient to carry the falling 80 stream of molten slag out of alignment with the entrance to the pouring gate and preferably into a position vertically above the top surface of the mold, which is not pierced by any of the various openings. The pre- 85 ferred procedure, because of the lightness of the crucible and because, in rail welding practice, it is usual to mount the crucible on a swinging arm, is to move the crucible aside slightly relatively to the mold just as 90 the last portions of the molten steel are being discharged from the crucible, so that the portion of the molten stream containing the slag will be diverted from the pouring gate and, if the slag is permitted to enter the 95 pouring gate at all, it will flow quietly over the upper surface of the mold into the gate without producing any surging of the highly fluid molten steel, which enters the gate, and, as a consequence, none of the slag will enter 100 the mold cavity proper.

What I claim is:

1. The method of preventing slag surging in thermite welding practice which comprises

deflecting the molten stream from the pouring gate of the mold approximately with the discharge of the final portion of the steel from the crucible.

- 5 2. The method of preventing slag surging in thermite welding practice which comprises teeming the molten metal directly into the

pouring gate of the mold and deflecting the molten stream containing the slag from the gate entrance by relative lateral movement <sup>10</sup> of the crucible and the mold.

In testimony whereof I affix my signature.

DONALD CAMERON DICKSON.